

## UNITED STATES PATENT OFFICE

2,191,033

COMPOSITION FOR THE TREATMENT OF  
SYNTHETIC WARP YARNSWendell G. Faw, Kingsport, Tenn., assignor to  
Eastman Kodak Company, Rochester, N. Y., a  
corporation of New JerseyNo Drawing. Application June 10, 1938,  
Serial No. 213,026

7 Claims. (Cl. 87—9)

This invention relates to the conditioning of textile yarns and more particularly to a method of and composition for the preparation of synthetic yarns composed of or containing organic derivatives of cellulose such as cellulose acetate, cellulose propionate, cellulose acetate propionate, cellulose acetate butyrate, and the like, to render them suitable for use in warping operations.

In the preparation of a warp for weaving, it is necessary to draw a large number of strands from individual packages through suitable guides, tension devices and spacers so that they converge and lie evenly spaced in one plane from which they can be wound onto a single beam. As is well known, synthetic yarns, particularly those composed of or containing organic derivatives of cellulose, are especially subject to the accumulation of charges of static electricity from frictional influences. This phenomenon is evidenced by the natural repulsion of many of the strands. This presents a serious problem especially when the tension is relieved by stopping the beaming operation.

It has been found to be absolutely necessary, not only to cut down friction by the application of a lubricant to the yarn, but also to employ an agent which will prevent the accumulation of static charges on the yarn. Many such de-electrification agents have been proposed. An especially successful class of anti-static agents is described and claimed in the co-pending application of J. R. Caldwell, Serial No. 114,085, filed December 3, 1936.

The problem of proper warp preparation does not end, however, with the provision of a satisfactory lubricant and a satisfactory anti-static or de-electrification agent. Several other factors enter into the problem and determine the quality of a satisfactory warp lubricant. To illustrate the complexity of the problem it is necessary to consider the various requirements which the yarn must meet in use. For example, after the yarn is drawn onto a beam in the warping process, it must be treated with a protective coating of a sizing material. To accomplish this, the yarn is passed through a bath consisting generally of a solution of gelatin and a softening agent such as Turkey red oil or glycerine and then is carried over suitable squeeze rolls and drying cylinders. In dry condition it is wound onto a beam for use in weaving. In the loom the yarn is subjected to severe abrasive action due to contact with the various moving parts of the loom. It is necessary, therefore, that the size coating be

sufficiently bonded to the yarn to provide adequate protection for the delicate filaments.

Taking as an example the difficulties inherent in the selection of a suitable anti-static agent, the anti-static may be, for example, of such a nature that it is too readily leached off the yarn by the size solution, thus allowing the yarn to accumulate static charges in passing over the drying cylinders and in subsequent steps of the process. The oil may resist the absorption of the size, thus necessitating the use of high concentrations of gelatin in the size bath with resultant additional cost and increased operating difficulties. Again, the oil may provide a poor bond between the size and the yarn, making necessary the application of heavier coatings to obtain a given required resistance to abrasion. For example, one oil may absorb 4% size, on the weight of the yarn, from a bath of given concentration, while another oil which has a poorer size absorption may result in a coating of only 3% size from the same bath. This would require a stronger bath to give the desired 4% size. Furthermore one oil may absorb 4% size, for example, and have the necessary resistance to abrasion, while another may absorb an equal amount of the size coating, but give only half the required protection, thus requiring heavier application for efficient weaving. It will thus be seen that the compounding of a suitable warp lubricant is a very complicated and difficult matter when one takes into consideration all of the different requirements such a lubricant has to fulfill in actual use and the necessary delicate balancing of one property against another.

This invention has as its principal object to provide an improved type of yarn-treating composition adapted for the treatment of synthetic warp yarns composed of or containing organic derivatives of cellulose such as cellulose acetate, cellulose propionate, cellulose acetate propionate, cellulose acetate butyrate and the like. A further object is to provide a warp lubricant which is capable of simultaneously lubricating and de-electrifying synthetic warp yarns and is also capable of giving the yarn good size absorption and providing a strong bond between the size coating and the yarn. Other objects will appear hereinafter.

These objects are accomplished by the following invention which, in its broader aspects, comprises the compounding of a warp yarn lubricant by mixing or blending a low viscosity textile mineral oil, a suitable anti-static agent or agents and a sulfonated oil of certain critical charac-

teristics. I have found that in order to meet all of the above-mentioned rigid requirements, one must employ a particular type of sulfonated oil, specifically, an oil having an SO<sub>3</sub> content of not over 5% and a moisture content of not over 10%. In addition I have found it is advantageous to employ a small amount of a blending agent such as a high molecular weight alcohol or a fatty acid to obtain a clear homogeneous mixture or 10 solution.

In the following examples and description I have set forth several of the preferred embodiments of my invention, but they are included merely for purposes of illustration and not as a 15 limitation thereof.

*Example I*

|                                                                          | Parts |
|--------------------------------------------------------------------------|-------|
| White mineral oil (viscosity 50 sec. Saybolt at 100° F.)                 | 50    |
| 20 Sulfonated olive oil SO <sub>3</sub> content 3.5% moisture content 9% | 25    |
| Triethanolamine salt of para toluene sulfonic acid                       | 10    |
| 25 Diethyl cyclohexylamine salt of sulfonated lauryl alcohol             | 10    |
| Oleyl alcohol                                                            | 5     |

*Example II*

|                                                                                        | Parts    |
|----------------------------------------------------------------------------------------|----------|
| 30 White mineral oil (viscosity 50-75 sec.)                                            | 40 to 60 |
| Sulfonated olive oil (SO <sub>3</sub> content below 5%, moisture content not over 10%) | 20 to 30 |
| Diethanolamine salt of dimethyl hydroxymethyl phosphonic acid                          | 5 to 25  |
| 35 Fatty acid or fatty alcohol                                                         | 0 to 10  |

*Example III*

|                                                                             | Parts |
|-----------------------------------------------------------------------------|-------|
| 30 Sulfonated olive oil (SO <sub>3</sub> content 3.5%, moisture content 9%) | 12    |
| 40 Monoethanolamine oleate                                                  | 12    |
| Pine oil alcohols                                                           | 8     |
| White mineral oil (50-60 sec. vis.)                                         | 62    |
| Monoethanolamine phosphate                                                  | 6     |

In the above examples I have referred to certain specific anti-static compounds. As indicated above, the compounds which I have found to be most suitable for the purposes of the present invention, of which the compounds mentioned in the examples are typical, are those described and claimed as anti-static agents in the copending application of J. R. Caldwell, Serial No. 114,085, filed December 3, 1936. The use of these compounds as anti-statics form no part of the present invention, except as they are used 45 in combination with other ingredients herein specified, but are the invention of J. R. Caldwell. These particular compounds are formed by the interaction of an organic base such as an alkylamine, a substituted alkylamine, an alicyclic 50 amine, an alkylolamine or an amine containing an ether linkage with a compound selected from the group consisting of the aromatic sulfonic acids, organic acids containing a cyclic ether residue and the organic acids containing an open 55 chain ether residue. Examples of such organic bases are amyl amine, diethyl amine, cyclohexylamine, monoethanolamine, triethanolamine, furfuryl amine, tetrahydrofurfuryl amine, beta-ethoxy ethylamine, etc. The aromatic sulfonic acid may contain a single aromatic nucleus, as in the case of benzenesulfonic acid, or it may be of the fused ring or polynuclear type as represented by the naphthalene sulfonic acids. The acids may be mono- or polysulfonic acids 70 and may contain other substituents in the nu-

cleus such as alkyl, hydroxyl and other groups. Among the compounds which have been found to be especially valuable are the salts formed by the interaction of the following: triethanolamine and benzene sulfonic acid, triethanolamine and toluene sulfonic acid, cyclohexylamine and paratoluene sulfonic acid, triethanolamine and sulfanilic acid, monoethanolamine and benzene sulfonic acid, monoethanolamine and toluene sulfonic acid, monoethanolamine and sulfanilic acid, ethylenediamine and benzene sulfonic acid, ethylenediamine and para-toluene sulfonic acid, monoethanolamine and 2-naphthanol-6-sulfonic acid, ethylenediamine and 2-naphthanol-6-sulfonic acid, ethylenediamine and sulfanilic acid, tetrahydrofurfurylamine and tetrahydrofuroic acid, cyclohexylamine and tetrahydrofuroic acid, etc.

As indicated above, the specific sulfonic compounds just referred to are very soluble in water and can be conveniently applied to the yarn, either in the form of aqueous solutions or aqueous emulsions. However, these sulfonic acid salts are insoluble in oils and tend to separate 25 from an oil-water mixture on the yarn and form another phase, this increasing the drag or friction of the lubricant.

Another class of compounds which are not only soluble in water, but also in mineral oils, 30 animal or vegetable glycerides and low melting waxes and which may be employed with even more satisfactory results than the water-soluble sulfonic compounds previously described includes 35 the salts formed by reacting an acid with an amine, the acid or the amine, or both, containing in their molecular structure one or more oxygen atoms combined in a saturated or unsaturated ether linkage. For example, the class of compounds derivable from the furans is especially 40 suitable as an oil-soluble type of anti-static lubricant, the furan or tetrahydrofuran residue when combined with an amino group to form a base, or with a carboxyl group to form an acid, greatly enhancing the solubility of the resulting 45 salts in oils.

Although salts formed from furoic acid show appreciable solubility in oils, it is more desirable to employ tetrahydrofuroic acid, as the structure of the latter compound more nearly approaches that of an aliphatic ether, and hence shows a greater tendency to dissolve in oils. Likewise, in the case of amines, tetrahydrofurfurylamine possesses the property of forming oil-soluble salts with both furoic and tetrahydrofuroic acids. Acids and amines containing open chain ether residues may also be used to advantage, as for example, methoxypropionic acid, ethoxybutyric acid, and beta-ethoxy ethylamine. For compounds of this type it is preferable to have four or more carbon atoms in the ether residue. Acids and amines having a molecular structure which embodies two or more ether linkages are also useful, as for example, dioxane acetic acid and beta-dioxane ethylamine.

The anti-static compounds may, as indicated above, be formed by reacting an acid containing an ether linkage, with a base (amine) containing an ether linkage, giving tetrahydrofurfurylamine tetrahydrofuroate; an acid containing no 70 ether linkage with an amine containing an ether linkage, giving tetrahydrofurfurylamine butyrate; an amine containing no ether linkage and preferably six or more carbon atoms, with an acid containing an ether linkage, giving cyclo- 75

hexylamine tetrahydrofuroate; an acid containing an unsaturated ether linkage with an amine containing a saturated ether linkage, giving tetrahydrofurfurylamine furoate.

5 It is to be understood that the compositions illustrated in the above specific examples are employed in the form of aqueous emulsions. The concentration of a given composition in the emulsion may vary between wide limits but I prefer to employ aqueous emulsions containing from 5-20% of the oil component based on the total weight of the emulsion.

10 The amount of the emulsion deposited on the yarn will also depend upon the particular type of yarn employed and the purpose for which the yarn is intended. For most warp yarns it is desirable to deposit a sufficient amount of the emulsion to give a residual oil content of 1% to 5%.

15 20 The emulsion may be deposited by any of the standard methods for applying yarn conditioning agents, such as by wick, roll, or submersion application, or otherwise.

25 As will be evident from the above description, the emulsions herein described may be applied to a wide variety of synthetic warp yarns, but are particularly effective in the conditioning of yarns composed of or containing organic acid esters of cellulose such as cellulose acetate. 30 Cellulose propionate, cellulose butyrate, cellulose acetate propionate, cellulose acetate butyrate and other single or mixed organic acid esters of cellulose as well as the cellulose ethers.

35 It should be emphasized that the effectiveness of the above described compositions in fulfilling the rigid requirements of a warp lubricant as specified above is attributable to the specific combination of ingredients employed in the formulas and particularly and fundamentally to the particular type of sulfonated olive oil which is employed. I have found after extensive experimentation that only by the use of sulfonated oil containing not over 5%  $\text{SO}_3$  and not over 10% moisture can a satisfactory anti-static warp lubricant of the type herein specified be obtained.

40 What I claim is:

1. A textile lubricating composition adapted for the treatment of synthetic warp yarns composed of or containing organic acid esters of cellulose and capable of simultaneously lubricating and de-electrifying the yarn and giving it the ability to absorb gelatin sizing compositions and to form a strong bond between the yarn and the size, which comprises a textile mineral oil, an anti-static agent, a sulfonated olive oil having an  $\text{SO}_3$  content of not over 5% and a moisture content of not over 10%.

45 2. A textile lubricating composition adapted for the treatment of synthetic warp yarns composed of or containing organic acid esters of cellulose and capable of simultaneously lubricating and de-electrifying the yarn and giving it the ability to absorb gelatin sizing compositions and to form a strong bond between the yarn and the size, which comprises a textile mineral oil, an anti-static agent, a sulfonated olive oil having an  $\text{SO}_3$  content of not over 5% and

a moisture content of not over 10%, and a blending agent.

3. The composition of claim 1 in which the anti-static agent is a salt formed by the interaction of an organic base selected from the group consisting of the alkyl amines, the substituted alkyl amines, the alicyclic amines, the alkylol amines and the amines containing an ether linkage with a compound selected from the group consisting of the aromatic sulfonic acids, the organic acids containing a cyclic ether residue and the organic acids containing an open chain ether residue.

10 4. The composition of claim 1 in which the anti-static component is a salt of an aliphatic amine and an organic sulfonic acid.

15 5. A textile lubricating composition adapted for the treatment of synthetic warp yarns composed of or containing organic acid esters of cellulose and capable of simultaneously lubricating and de-electrifying the yarn and giving it the ability to absorb gelatin sizing compositions and to form a strong bond between the yarn and the size, having the following formula:

|                                                                         | Parts |
|-------------------------------------------------------------------------|-------|
| White mineral oil (viscosity 50 sec. Saybolt at 100° F.)                | 50    |
| Sulfonated olive oil ( $\text{SO}_3$ content 3.5%, moisture content 9%) | 25    |
| Triethanolamine salt of para toluene sulfonic acid                      | 30    |
| Diethyl cyclohexylamine salt of sulfonated lauryl alcohol               | 10    |
| Oleyl alcohol                                                           | 10    |
|                                                                         | 5     |
|                                                                         | 35    |

20 6. A textile lubricating composition adapted for the treatment of synthetic warp yarns composed of or containing organic acid esters of cellulose and capable of simultaneously lubricating and de-electrifying the yarn and giving it the ability to absorb gelatin sizing compositions and to form a strong bond between the yarn and the size, having the following formula:

|                                                                                       | Parts    |
|---------------------------------------------------------------------------------------|----------|
| White mineral oil (viscosity 50-75 sec.)                                              | 40 to 60 |
| Sulfonated olive oil ( $\text{SO}_3$ content below 5%, moisture content not over 10%) | 20 to 30 |
| Diethanolamine salt of dimethyl hydroxymethyl phosphonic acid                         | 5 to 25  |
| Fatty acid or fatty alcohol                                                           | 0 to 10  |
|                                                                                       | 50       |

25 7. A textile lubricating composition adapted for the treatment of synthetic warp yarns composed of or containing organic acid esters of cellulose and capable of simultaneously lubricating and de-electrifying the yarn and giving it the ability to absorb gelatin sizing compositions and to form a strong bond between the yarn and the size, having the following formula:

|                                                                         | Parts |
|-------------------------------------------------------------------------|-------|
| Sulfonated olive oil ( $\text{SO}_3$ content 3.5%, moisture content 9%) | 12    |
| Monoethanolamine oleate                                                 | 12    |
| Pine oil alcohol                                                        | 8     |
| White mineral oil (50-60 sec. visc.)                                    | 62    |
| Monoethanolamine phosphate                                              | 6     |

WENDELL G. FAW.